

Patented July 2, 1929.

1,719,167

## UNITED STATES PATENT OFFICE.

GEORGE D. CHAMBERLAIN, OF ASHLAND, KENTUCKY, ASSIGNOR TO R. T. VANDER-BILT COMPANY, INCORPORATED, OF NEW YORK, N. Y., A CORPORATION OF NEW YORK.

## CLEANING OF METALS, ETC.

No Drawing.

Application filed January 11, 1927. Serial No. 160,526.

This invention relates to the pickling and cleaning of metals, and particularly to the pickling of iron or steel, to remove scale therefrom, although the invention is of more or 5 less general application to the cleaning or pickling of metals such as iron or steel for the removal of oxides or scale therefrom.

The pickling or cleaning of iron or steel is commonly effected by means of acid pickling 10 or cleaning baths which dissolve the scale or oxide from the metal. The pickling baths commonly employed are acid baths which often attack the metal as well as the scale. This action on the metal is undesirable and 15 objectionable, involving not only excessive consumption of acids, but also corrosion or dissolving of metal and tending to give a rough or pitted surface.

The present invention provides an improved bath for pickling or cleaning iron or 20 steel and also an improved process of pickling or cleaning the metal in which the acid pickling bath has incorporated therein a small amount of a condensation product of a nitrogenous base with a ketone.

I have found that the addition of a small amount of a suitable condensation product of a nitrogenous base with a ketone prevents or 25 retards or inhibits the attack of the acid pickling bath on the metal without interfering with the removal of scale or oxide by the acid bath.

The agents which are added to the cleaning or pickling bath, according to the present invention, include various condensation products of nitrogenous bases with ketones.

Among these may be mentioned condensation products of various nitrogenous bases, such as ammonia and certain amines, for example 30 hydroxyl amine. Certain condensation products of nitrogenous bases with acetone are particularly advantageous such as the condensation product of acetone with ammonia.

A suitable method of making the condensation product of acetone with ammonia is to 45 introduce ammonia gas into acetone containing powdered calcium chloride in suspension until the acetone is saturated, and then allowing the reaction mixture to stand until the 50 reaction is completed. The resulting oily product can be freed from excess acetone and ammonia by distillation, and can be further treated to separate the different acetone amine products or fractions therefrom. Condensa-

tion products of other nitrogenous bases and 55 ketones may be formed in a similar manner, using other nitrogenous bases and ketones as starting products.

The acid pickling baths with which the agents mentioned are used may be acid baths 60 such as are commonly employed for pickling or cleaning iron and steel, containing for example, about 10% of sulfuric acid. Such baths are gradually impoverished by the action of the acid in removing the scale or 65 rust and their content of ferrous sulfate increases until the bath becomes too weak or too concentrated in ferrous sulfate for further use. Instead of using sulfuric acid baths, other acid baths can be used, includ- 70 ing acid sulfate baths.

The amount of the condensation product added to the bath for carrying out the pickling or cleaning operation can be varied. In general, only a small amount of the condensation product is required, for example, 75 a small fraction of one percent. In the case of the condensation product of acetone with ammonia, for example, about two pounds of the condensation product can be employed 80 for each ton of 60 degree acid used in the pickling bath. The condensation product employed should be one which is stable and does not decompose to any objectionable extent in the acid bath.

The carrying out of the pickling or cleaning operation may be the same as in ordinary practice. For example, the pickling can be carried out continuously by passing the material to be pickled, such as wire or sheets, 90 through a number of baths in a regulated manner; or by immersing the article to be pickled in the pickling bath for a suitable period of time. The temperature of the bath can be varied, ordinarily being around 150 or 180° F. 95 The pickling bath may be replenished by the addition of further amounts of acid until the iron sulfate reaches too great a concentration.

The addition of the condensation product to the bath prevents or retards or inhibits the action of the acid bath on the metal without interfering with the removal of scale or oxide. The formation of hydrogen by the action of the acid bath on the metal is also reduced and the evolution of acid mist or fumes also greatly reduced. There is also a saving in the acid as well as a protection of the metal. The reduced amount of action of the acid on the

148

metal and the reduction in amount of hydrogen produced correspondingly reduces the amount of hydrogen absorbed by the metal.

The employment of the condensation product in the pickling or cleaning operation, according to the present invention, involves but small additional expense and results in advantages in operation, economy of acid, protection of the metal from attack, etc., which 10 materially improve the pickling and cleaning operation.

In the claims, the formula  $\text{NH}_2\text{R}$  is used to indicate a nitrogenous base in which the R may be H or may be a radical which, with the 15  $\text{NH}_2$  group, forms an amine such as hydroxyl amine.

I claim:

1. The method of cleaning or pickling metals which comprises subjecting the same to 20 a non-oxidizing mineral acid pickling or cleaning bath and inhibiting the chemical action of the acid on the metal without interfering with the removal of scale or oxide, and thereby reducing the formation of hydrogen and the production of acid fumes and effecting an economy in the acid consumed, by incorporating in the acid bath a small amount of a condensation product of a nitrogenous base with a ketone.

30 2. The method of cleaning or pickling metals which comprises subjecting the same to a non-oxidizing mineral acid pickling or cleaning bath and inhibiting the chemical action of the acid on the metal without interfering 35 with the removal of scale or oxide, and thereby reducing the formation of hydrogen and the production of acid fumes and effecting an economy in the acid consumed, by incorporating in the acid bath a small amount 40 of a condensation product of acetone with a compound of the formula  $\text{NH}_2\text{R}$ .

3. The method of cleaning or pickling metals which comprises subjecting the same to a non-oxidizing mineral acid pickling or 45 cleaning bath and inhibiting the chemical action of the acid on the metal without interfering with the removal of scale or oxide, and thereby reducing the formation of hydrogen and the production of acid fumes and effecting an economy in the acid consumed, by incorporating in the acid bath a small 50 amount of a condensation product of acetone with ammonia.

4. The method of pickling or cleaning iron 55 or steel which comprises subjecting the same to an acid pickling bath containing sulfuric acid and inhibiting the chemical action of the acid on the metal without interfering with the removal of scale or oxide, and thereby reducing the formation of hydrogen and the 60 production of acid fumes and effecting an economy in the acid consumed, by incorporat-

ing in the acid bath a small fraction of one percent of a condensation product of a nitrogenous base with a ketone.

65

5. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid fumes and effecting an economy in the acid consumed, by incorporating in the acid bath a small fraction of one 75 percent of a condensation product of acetone with a compound having the formula  $\text{NH}_2\text{R}$ .

6. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid fumes and effecting an 80 economy in the acid consumed, by incorporating in the acid bath a small fraction of one percent of a condensation product of acetone with ammonia.

7. A non-oxidizing mineral acid bath for 90 pickling or cleaning metals which contains a small amount of a condensation product of a nitrogenous base with a ketone.

8. A non-oxidizing mineral acid bath for pickling or cleaning metals which contains a 95 fraction of one percent of a condensation product of acetone with a nitrogenous base.

9. A bath for pickling or cleaning iron or steel which comprises sulfuric acid and a 100 small amount of a condensation product of acetone with a nitrogenous base.

10. A bath for pickling or cleaning iron or steel which comprises sulfuric acid and a fraction of one percent of a condensation product of acetone with ammonia.

105

11. A bath for pickling or cleaning iron or steel which comprises sulfuric acid and a condensation product of a nitrogenous base with a ketone.

12. A bath for pickling or cleaning iron or 110 steel which comprises sulfuric acid and a condensation product of acetone with ammonia.

13. A non-oxidizing mineral acid bath for pickling or cleaning metals which contains a 115 condensation product of acetone with a nitrogenous base.

14. A non-oxidizing mineral acid bath for pickling or cleaning metals which contains a condensation product of acetone with ammonia.

120

In testimony whereof I affix my signature.

GEORGE D. CHAMBERLAIN.